

## UNITED STATES PATENT OFFICE

2,526,544

## METHOD OF PRODUCING A METALLIC COATING ON MAGNESIUM AND ITS ALLOYS

Herbert K. De Long, Midland, Mich., assignor to  
The Dow Chemical Company, Midland, Mich.,  
a corporation of Delaware

No Drawing. Application October 6, 1947,  
Serial No. 778,283

9 Claims. (Cl. 117—130)

1

The invention relates to the surface treatment of articles of magnesium and magnesium-base alloys containing upwards of 85 per cent of magnesium. It more particularly concerns a surface treatment method for the aforesaid metals which promotes the adherence thereto of metallic coatings, particularly those produced by electrodeposition.

Articles of magnesium and its alloys are among the most difficult of all common structural metals to provide with an adherent metallic coating of another metal. A number of methods have been proposed heretofore by which coatings of certain metals may be provided on articles of magnesium and its alloys. However, the coatings obtained are not wholly satisfactory either from the standpoint of adhesion, appearance, or protection afforded the underlying metal, and, in some instances, the coating procedures are complex and difficult to perform. It is a desideratum in the art to provide a method of treatment by which a magnesium or magnesium-base alloy article may be given an adherent coating of another metal, and particularly an adherent metallic coating which is either or both protective and decorative.

Accordingly, it is the principal object of the invention to provide a method fulfilling this need. A particular object is to provide a method of treating the surface of an article of a magnesium or magnesium-base alloy, whereby adherent electroplates of other metals thereon may be obtained. Other objects and advantages of the invention will appear as the description of the invention proceeds.

Briefly the method contemplated by the invention comprises treating the cleaned article of magnesium or magnesium-base alloy with an alkaline aqueous solution containing pyrophosphate and zinc solution, whereby a zinc coating is deposited upon the metal. The zinc coated surface obtained is used as a base for the retention of other metallic coatings particularly those deposited thereon by electrodeposition, as from an alkaline cyanide aqueous electroplating bath. These electroplates may be used as the base for still other metallic coatings, such as those which cannot be deposited directly on zinc or magnesium.

Prior to carrying out the method, the surface of the article is cleaned in a manner to leave the surface free from contamination and in a condition whereby the metal will react with the zincing solution, of dissolved pyrophosphate and zinc, to bring about the deposition of the zinc coating. The surface of the article may be pre-

2

pared for zincing by a mechanical cleaning such as machining, wire brushing, buffing, and the like, or by a chemical treatment with solvents or pickling agents, the method used being chosen in accordance with the nature of the surface to be cleaned and smoothness desired. While mechanical cleaning usually leaves the surface in a condition capable of reacting with the zincing solution, chemical treatment, such as the conventional pickling operations leave an oxidic film which interferes with the action of the zincing solution.

I have found that the oxidic film, however formed, should be removed before proceeding with the method of the invention. For the removal of the film or coating, the article may be immersed in a film removing solution such as a 2 per cent solution of acetic acid in water or a 1 per cent solution of hydrochloric acid in water. Still better results as regards the adhesion of the zinc coating subsequently to be applied are obtained when an aqueous solution of aluminum chloride is used to remove the film left by other pickling solutions or solvent treatments. The aluminum chloride solution may contain from about 5 to 250 grams or more of  $AlCl_3$  per liter, or preferably from about 80 to 165 grams per liter. A generally useful concentration is about 110 grams of  $AlCl_3$  per liter, the article to be treated being immersed in the solution for about a minute although other times may be used. Treatment of an article of magnesium and its alloys in an aqueous solution of aluminum chloride has special advantages and is more fully set forth in my copending application, Serial No. 778,282, filed October 6, 1947 issued as Patent No. 2,499,269 on February 28, 1950.

In carrying out the method of the invention, the article to be zinc coated is treated with an aqueous zincing bath having a pH between about 8 to 11 and comprising zinc and pyrophosphate solution as aforesaid, as by immersing the article in the bath, the article and treating solution being maintained in contact until a coating of metallic zinc is deposited on the surface of the article. Formation of the coating is visually evident by its uniform grey color and appears to result from the reducing action of the metallic magnesium of the surface of the article on the dissolved zinc in the zinc-pyrophosphate solution, whereby the reduced zinc is deposited in situ, the reduction proceeding according to the equation:



55 A number of formulations of the zinc-pyrophosphate bath have been found effective to

deposit the zinc coating of which the following are illustrative:

*Example 1*

|                                                | Grams |
|------------------------------------------------|-------|
| Sodium pyrophosphate ( $Na_4P_2O_7$ )          | 10    |
| Zinc fluoride ( $ZnF_2$ )                      | 1.5   |
| Water sufficient to make 100 grams of solution |       |

The pH of the solution is about 9.6.

*Example 2*

|                                                | Grams |
|------------------------------------------------|-------|
| Sodium pyrophosphate                           | 10    |
| Zinc sulfate ( $ZnSO_4 \cdot 7H_2O$ )          | 4     |
| Sodium fluoride ( $NaF$ )                      | 0.5   |
| Water sufficient to make 100 grams of solution |       |

The pH of the solution is about 10.2.

*Example 3*

|                                                | Grams |
|------------------------------------------------|-------|
| Sodium pyrophosphate                           | 10    |
| Zinc fluoride                                  | 1     |
| Ferric fluoride ( $FeF_3$ )                    | 0.01  |
| Water sufficient to make 100 grams of solution |       |

The pH of solution is about 9.8.

*Example 4*

|                                                | Grams |
|------------------------------------------------|-------|
| Potassium pyrophosphate ( $K_4P_2O_7$ )        | 10    |
| Zinc fluoride                                  | 0.5   |
| Sodium fluoride                                | 2     |
| Water sufficient to make 100 grams of solution |       |

The pH of the solution is about 9.6.

*Example 5*

|                                                | Grams |
|------------------------------------------------|-------|
| Sodium pyrophosphate                           | 6     |
| Zinc cyanide ( $Zn(CN)_2$ )                    | 1     |
| Sodium fluoride                                | 2     |
| Water sufficient to make 100 grams of solution |       |

The pH of the solution is about 10.6.

*Example 6*

|                                                | Grams |
|------------------------------------------------|-------|
| Sodium pyrophosphate                           | 6.0   |
| Zinc cyanide                                   | 1.0   |
| Sodium fluoride                                | 0.5   |
| Ferric oxalate ( $FeC_2O_4 \cdot 2H_2O$ )      | 0.005 |
| Water sufficient to make 100 grams of solution |       |

The pH of the solution is about 10.6.

The foregoing solutions are used preferably at their boiling temperature, the article to be treated being immersed therein for about 1 to 30 minutes or longer, although 3 to 7 minutes immersion is preferred. The coating obtained is generally not over 0.0001 inch thick and cannot be peeled off.

Other alkali metal pyrophosphates may be used, such as those of lithium, rubidium, and cesium. If desired, the pyrophosphate in the bath may be provided by adding pyrophosphoric acid to the bath and sufficient alkali of the alkali metal family to raise the pH to the alkaline side, thereby in effect producing an alkali metal pyrophosphate in solution as an active ingredient. The zinc in solution may be derived from various soluble zinc compounds, in addition to those in the foregoing examples, such as zinc acetate, zinc borate, zinc bromide, and zinc chloride.

The concentration of the pyrophosphate and zinc in solution, effective for producing the zinc coating, does not appear to be critical and a wide variation in their concentrations is permissible. In the case of the pyrophosphate, the concentration of  $P_2O_7$  may be from about 0.6 to 27.0 grams, and the concentration of Zn from about 0.1 to 4.0

grams per 100 grams of solution, although other proportions may be used. Pyrophosphoric acid and various alkalies, such as an alkali metal hydroxide or carbonate, may be used to adjust the pH of the zinc plating solution to the desired value, if necessary.

While the presence of dissolved fluoride, derived from a soluble metal fluoride (preferably an alkali metal fluoride), in the zinc plating bath is preferred because it reduces the time of treatment and results in better adhesion of the zinc, its presence is not essential and may be omitted, if desired, provided the bath contains the ions of pyrophosphate and zinc and the pH is between about 8 and 11. A suitable fluorine concentration is between about 0.25 and 8 per cent, although other concentrations may be used.

Although the pyrophosphate-zinc bath is used preferably while at or about the boiling point, lower temperatures may be used but the rate of zinc deposition is slower. At 20° to 25° C., for example, a zinc coating is obtained which appears to reach a maximum thickness in about 30 minutes; while at the boiling point or near 100° C., a similar coating is obtained in about 1 minute.

In forming the coating, there is a mild gassing at the surface of the immersed article especially at first and this gassing diminishes as the coating action proceeds. On attaining its ultimate thickness, the reaction appears to cease and little or no gassing is observed. The article need not be left in the bath beyond the stage when gassing ceases or nearly ceases.

Another indication that the zinc coating operation has proceeded to a limiting extent is that the surface undergoing plating becomes uniformly grey in appearance. It is to be understood that useful coatings are obtained in less time than that required for the coating action to come to an apparent end, as when gassing ceases, or nearly ceases, or when the article becomes uniformly grey.

Immersion of the article in the zinc plating solution is the preferable way of maintaining contact between the solution and the surface to be coated, but other ways of maintaining contact may be used such as spraying the solution onto the surface of the article. After the treatment, the plated article is thoroughly rinsed in water.

The zinc coating obtained by the foregoing method, referred to hereinafter sometimes as a "contact coating," has utility as a protection and decoration, and, if desired, the coated article need not be further treated except to dry it. However, the zinc contact coating has the unique advantage of being capable of receiving adherent deposits of other metals in similar manner to that of zinc itself. For example, the contact coating before drying may be electroplated in conventional cyanide alkaline plating baths suitable for electroplating zinc. Various metals may be thus deposited from their alkaline electroplating baths, e. g. silver, copper, gold, cadmium, tin, and various combinations of these metals.

In providing an electroplating over the contact coating, the coated article is preferably given a strike from a cyanide plating bath, for example, a copper strike from an alkaline copper plating bath, such as a conventional copper cyanide plating bath. In carrying out the electroplating operation, the contact coated article is transferred directly to the plating bath while the ar-

tic is still wet from the rinsing step following the application of the contact coating as described, and a strike is produced over the zinc contact coating, the article being the cathode as in conventional plating practice.

An example of a suitable alkaline copper electroplating bath is the following:

|                                                                                    | Grams |
|------------------------------------------------------------------------------------|-------|
| Copper cyanide (CuCN)                                                              | 41.3  |
| Sodium cyanide (NaCN)                                                              | 50.8  |
| Sodium carbonate (Na <sub>2</sub> CO <sub>3</sub> )                                | 30.0  |
| Rochelle salt (KNaC <sub>4</sub> H <sub>4</sub> O <sub>6</sub> ·4H <sub>2</sub> O) | 45.0  |

Other conventional alkaline cyanide plating baths may be used, such as those of the aforementioned metals, although for the purpose of obtaining a strike, the copper plating bath is preferred. In forming a copper deposit using the above bath, it is operated, preferably at a temperature of about 150° F. A current density of about 5 to 10 amperes per square foot of surface is maintained for about 3 minutes or longer and then raised to about 15 to 20 amperes per square foot for 2 minutes longer. This treatment results in coating the zinced surface with a layer of copper that adheres well and covers the zinc. If desired, the copper plating operation may be continued for a longer time to produce a heavier coating and other current densities and plating temperature may be used as known in the electroplating art.

Having applied a strike of copper or other metal coating over the contact coating, it is possible to further electroplate the article with any other metal that is capable of being electrodeposited upon the strike coating. For example, I have found that cadmium, chromium, nickel, silver, and zinc or combinations of metals can be electroplated in conventional manner on the electroplated contact coating.

Among the advantages of the method are that by either contact coating the magnesium (or magnesium alloy) article with zinc or electroplating the zinc contact coated article, it is possible to provide a finish coating of any metal that is capable of electrodeposition from a conventional plating bath. As already indicated, for example, the cyanide plating bath may be used for electroplating over zinc (deposited by contact coating or plating as described or electrolytically over the contact coating) any of the various metals that can be plated on zinc from such baths. Furthermore, by choosing as the metal to be deposited from the cyanide bath one over which a plating may be deposited from an acid plating bath, for example, the metal copper, all the metals which are capable of being applied as electroplates from either a conventional acid or alkaline plating bath, may be deposited upon articles of magnesium and its alloys as a finish coating.

For example, metals such as chromium and nickel which cannot be plated directly on magnesium or zinc, because of the acid nature of their plating baths, can be readily electroplated as a finish coating on a magnesium and magnesium alloy article from the conventional electroplating baths of these metals after the article is zinc contact coated according to the invention and plated from an alkaline bath with a metal resistant to acid plating baths.

I claim:

1. In a method of forming an adherent metallic coating upon the surface of an article of magnesium and its alloys, the step which comprises

treating the surface of the article with an alkaline aqueous solution having a pH between about 8 and 11 and consisting essentially of water, an alkali metal pyrophosphate, and a water-soluble zinc salt selected from the group consisting of zinc acetate, zinc borate, zinc bromide, zinc chloride, zinc cyanide, zinc fluoride, zinc sulfate, the concentration of the pyrophosphate radical being between 0.6 and 27 grams and that of the zinc being between 0.1 and 4 grams per 100 grams of the solution, whereby a coating of metallic zinc is deposited in situ on the surface of the article.

2. In a method of forming an adherent metallic coating upon the surface of an article of magnesium and its alloys, the step which comprises treating the surface of the article with an alkaline aqueous solution having a pH between about 8 and 11 and consisting essentially of water, an alkali metal pyrophosphate, and a water-soluble zinc salt selected from the group consisting of zinc acetate, zinc borate, zinc bromide, zinc chloride, zinc cyanide, zinc fluoride, zinc sulfate, the concentration of the pyrophosphate radical being between 0.6 and 27 grams and that of the zinc being between 0.1 and 4 grams per 100 grams of the solution and, the temperature of the solution being between about 20° C. and its atmospheric boiling point, whereby a coating of metallic zinc is deposited in situ on the surface of the article.

3. In a method of forming an adherent metallic coating upon the surface of an article of magnesium and its alloys, the step which comprises treating the surface of the article with an alkaline aqueous solution having a pH between about 8 and 11 and consisting essentially of water, an alkali metal pyrophosphate, a water-soluble zinc salt selected from the group consisting of zinc acetate, zinc borate, zinc bromide, zinc chloride, zinc cyanide, zinc sulfate, the concentration of the pyrophosphate radical being between 0.6 and 27 grams and that of the zinc being between 0.1 and 4 grams per 100 grams of the solution, and a water-soluble metal fluoride in amount between about 0.25 and 8 grams per 100 grams of the solution, whereby a coating of metallic zinc is deposited in situ on the surface of the article.

4. In a method of forming an adherent metallic coating upon the surface of an article of magnesium and its alloys, the step which comprises treating the surface of the article with an alkaline aqueous solution having a pH between about 8 and 11 and consisting essentially of water, an alkali metal pyrophosphate in amount sufficient to furnish 0.6 to 27 grams of pyrophosphate radical per 100 grams of the solution, zinc sulfate in amount sufficient to furnish 0.1 to 4 grams of zinc per 100 grams of the solution, and a water-soluble metal fluoride in amount sufficient to furnish between 0.25 and 8 grams of fluoride per 100 grams of solution.

5. In a method of forming an adherent metallic coating upon the surface of an article of magnesium and its alloys, the step which comprises treating the surface of the article with an alkaline aqueous solution having a pH between about 8 and 11 and consisting essentially of water, an alkali metal pyrophosphate in amount sufficient to furnish 0.6 to 27 grams of pyrophosphate radical per 100 grams of the solution and zinc fluoride in amount sufficient to furnish 0.1 to 4.0 grams of zinc per 100 grams of solution,

whereby a coating of metallic zinc is deposited in situ on the surface of the article.

6. In a method of forming an adherent metallic coating upon the surface of an article of magnesium and its alloys, the step which comprises treating the surface of the article with an alkaline aqueous solution having a pH between about 8 and 11 and consisting essentially of water, an alkali metal pyrophosphate in amount sufficient to furnish 0.6 to 27 grams of pyrophosphate radical per 100 grams of the solution, zinc fluoride in amount sufficient to furnish 0.1 to 4.0 grams of zinc per 100 grams of solution, and ferric fluoride in amount sufficient to furnish 0.25 to 8 grams of fluoride per 100 grams of solution, whereby a coating of metallic zinc is deposited in situ on the surface of the article.

7. In a method of forming an adherent metallic coating upon the surface of an article of magnesium and its alloys, the step which comprises treating the surface of the article with an alkaline aqueous solution having a pH between about 8 and 11 and consisting essentially of water, an alkali metal pyrophosphate in amount sufficient to furnish 0.6 to 27 grams of pyrophosphate radical per 100 grams of the solution, zinc fluoride in amount sufficient to furnish 0.1 to 4.0 grams of zinc per 100 grams of solution, and sodium fluoride in amount sufficient to furnish 0.25 to 8 grams of fluoride per 100 grams of solution, whereby a coating of metallic zinc is deposited in situ on the surface of the article.

8. In a method of forming an adherent metallic coating upon the surface of an article of magnesium and its alloys, the step which comprises treating the surface of the article with an alkaline aqueous solution having a pH between about 8 and 11 and consisting essentially of water, sodium pyrophosphate in amount sufficient to provide 0.6 to 27 grams of pyrophosphate radical per 100 grams of the solution,

zinc cyanide in amount sufficient to provide 0.1 to 4.0 grams of zinc per 100 grams of the solution, and sodium fluoride in amount sufficient to provide 0.25 to 8 grams of fluoride per 100 grams of the solution, whereby a coating of metallic zinc is deposited in situ on the surface of the article.

9. In a method of forming an adherent metallic coating upon the surface of an article of magnesium and its alloys, the step which comprises treating the surface of the article with an alkaline aqueous solution having a pH between about 8 and 11 and consisting essentially of water, sodium pyrophosphate in amount sufficient to furnish 0.6 to 27 grams of pyrophosphate radical per 100 grams of the solution, zinc cyanide in amount sufficient to furnish 0.1 to 4 grams of zinc per 100 grams of the solution, sodium fluoride in amount sufficient to furnish 0.25 to 8 grams of fluoride per 100 grams of the solution, and ferrous oxalate, whereby a coating of metallic zinc is deposited in situ on the surface of the article.

25 HERBERT K. DE LONG.

#### REFERENCES CITED

The following references are of record in the file of this patent:

#### UNITED STATES PATENTS

| Number    | Name     | Date           |
|-----------|----------|----------------|
| 744,170   | Darlay   | Nov. 17, 1903  |
| 1,607,676 | Jirotka  | Nov. 23, 1926  |
| 1,627,900 | Hewitson | May 10, 1927   |
| 1,801,629 | Kenaga   | Apr. 21, 1931  |
| 2,297,241 | Perner   | Sept. 29, 1942 |
| 2,313,756 | Loose    | Mar. 16, 1943  |
| 2,419,190 | Wagoner  | Apr. 15, 1947  |

#### OTHER REFERENCES

Iron Age, September 20, 1888, page 424.